

H. Rowe.

Fagot for Railroad Rails.

No 77,659.

Patented May 5, 1868.

Fig 1



Fig 2



Fig 3.



Fig 4.



Witnesses.

David Harry

James Park

Inventor.

Harrison Rowe.

# UNITED STATES PATENT OFFICE.

HARRISON ROWE, OF MARIETTA, PENNSYLVANIA.

## IMPROVED FAGOT FOR RAILROAD-RAILS.

Specification forming part of Letters Patent No. 77,659, dated May 5, 1868.

*To all whom it may concern :*

Be it known that I, HARRISON ROWE, of Marietta, in the county of Lancaster and State of Pennsylvania, have invented a new and Improved Mode for Making up the Pile or Fagot for being Rolled into Rails for Railroads; and I do hereby declare that the following is a full and exact description thereof, reference being had to the accompanying drawings, making a part of this specification, in which—

Figure 1 is a perspective (abridged) view of the pile ready for rolling; Fig. 2 is an end view of the same. Fig. 3 shows the form of a B-shaped or filling-in plate; Fig. 4, a reduced figure of the rail, the difference in its composition indicated.

The nature of my invention consists in the formation and application of a top and bottom plate expressly rolled wider than the intermediate filling or pile, which consists of two pairs of old rails cut to length, laid on their sides, their tread in close contact, with two B-plates between said pairs, and with a similar B-shaped plate on top and bottom, forming a square pile, between the top and bottom plates, of flat and wider bars.

To enable others skilled in the art to make and use my invention, I will proceed to describe the several preparatory stages.

First, for the top plate or plates A of the pile, a flat bar of the desired width and thickness is rolled out of hard granular iron and cut to length. A flange may be made on each side of the under face of the bar A; marked a, Fig. 2, to lock against the outside of the flanges of the upper pair of rails, c, in order to extend and more effectually bind the parts together under the rollers, so constructed as to crowd the said lap or flange a over and into the flange of the rail C. To form the flat bar E for the bottom of the pile, I first make a flat bar as follows: I take strong cold-short or neutral iron rolled into a bar of the desired width and thickness, cut to length for both a top and bottom of a pile, filled in between them with short pieces of old rails C, B-iron D, of good fibrous iron, of any shape so as to form a pile between the two plates. This pile is brought to a welding-heat and rolled edgewise into a bar of the desired width and thickness, so as to bring the cold-short or neutral iron to the outer edges, e, of the bar, forming the bottom plate E of the pile, Fig. 1. This is to prevent the

flange from cracking or tearing when rolled into a rail.

I use two kinds of plates for filling in. The upper B-plate B is made of puddled iron. The other B-plates D are made out of crooked ends, cross-ends, old rails, or any kind of iron, mixed with puddled iron or otherwise. Fig. 3 shows one of those B-plates. Figs. 1 and 2 show their employment in building the pile or fagot, in combination with the two pairs of rails c c c, with their flanges, forming the flat sides between the top and bottom plates, A E. This pile is subjected to heat and rolled out into rails in the usual manner. By substituting a steel bar for A with the proper flux the same pile could be rolled into steel-capped rails, and yet differ substantially from the Patent No. 43,593, in which a central pair of rails are joined by their flange or base with a pair above and below with their flanges outside, and the tread widely separated, using also a corrugated top and bottom plate made with two grooves, leaving open corners and larger interior spaces, not calculated to make a solid and uniform rail.

I am aware also that in the Reissue No. 2,697, in which are corrugated steel slabs (equivalent to my B-plate B) or form pieces, does not alter the case, differing substantially in combination and result. By my method of piling I do not only save the reworking of the old rails by blooming or reheating them, but secure a better consolidated head or tread, be it steel-capped or of strong granular iron, by means of my wider or overlapping top bar A, as I also secure a better flange and in every respect a superior rail.

I am further aware that various methods are employed in making up the fagot or pile; but I am not aware that my mode was ever (substantially) employed by providing an overlapping top or flange, a, in piling for the purpose named.

What I claim as my invention, and desire to secure by Letters Patent, is—

The manner of making and applying my wider top and bottom plates, A E, in combination with the intermediate filling, B C D, when made into a pile or fagot for being rolled into rails for railroads, substantially in the manner specified.

HARRISON ROWE.

Witnesses:

JAMES PARK,  
DAVID HARRY.